

# United States Patent Office

2,939,774

Patented June 7, 1960

1

2,939,774

## MOTOR FUEL COMPOSITIONS

Paul E. Oberdorfer, Jr., Claymont, Del., assignor to Sun Oil Company, Philadelphia, Pa., a corporation of New Jersey

No Drawing. Filed Mar. 6, 1957, Ser. No. 644,221

9 Claims. (Cl. 44—63)

This invention relates to improved motor fuel compositions, and more particularly to a motor fuel containing a small amount of a cyclic carbonate inner ester, sufficient to substantially reduce engine deposits.

In the operation of internal combustion engines, whether of the spark ignition or compression ignition type, carbonaceous deposits tend to form in the combustion chambers. In the case of spark ignition engines the problem is serious, since the deposits tend to cause knock, thus increasing the octane number requirement of the engine, and also the carbonaceous material in the deposits has a tendency to burn at low temperatures to form incandescent particles on the combustion chamber walls which cause surface ignition. In compression ignition engines the problem of knock does not occur, but the deposits are undesirable because they tend to clog up the fuel injection nozzle.

It is the object of the present invention to provide a liquid fuel for internal combustion engines effective to reduce the amount of engine deposits, and which is also effective to raise the ignition temperature of such deposits as are formed to a value high enough to prevent the formation of incandescent particles in the combustion chamber, thereby eliminating knock due to surface ignition.

I have found that the foregoing objective may be attained if a small quantity of a cyclic carbonate inner ester having the formula:



in which each R may be hydrogen or a hydrocarbon radical, but at least one R is a hydrocarbon radical, is added to a liquid hydrocarbon fuel. Preferred esters are propylene carbonate:



or the butylene carbonates:



Higher molecular weight carbonates may also be used, such as amylene carbonate and higher homologues, and aromatic carbonates such as phenylethylene carbonate

2

and its homologues, but since the effectiveness of the additive is apparently due solely to the:



group, they are not preferred, since a greater amount of the ester must be used to produce the same effect. In general, the ester should preferably be added to the fuel in an amount of from about 0.02% by weight to about 2.0% by weight, although percentages above and below this range may be used. If the fuel is to be used with a clean engine, percentages in the lower part of this range should be used, while if it is desired to use the fuel in an engine which has already accumulated carbonaceous deposits, percentages in the higher portion of the range should be used.

In order to demonstrate the results which may be obtained with the fuels of the present invention, the following examples are given:

### EXAMPLE I

In this test a 1956 Cadillac engine was used. The test was started on fuel without the additive of the present invention, and the engine was run for a period of 219 hours in order to build up a substantial amount of engine deposits, after which a fuel admixed with 1% propylene carbonate was used. The engine was connected to a dynamometer under a load such that it would take 11 seconds at full throttle to accelerate from idle to 2500 r.p.m. The fuels used were rated according to their performance number, which is related to octane number according to the following equations:

$$(Below 100 O.N.) \text{ Octane No.} = 128 - \frac{2800}{\text{Performance No.}}$$

$$(Over 100 O.N.) \text{ Octane No.} = \frac{100 + \frac{2800}{\text{Performance No.}} - 100}{3}$$

Performance number was used because it is more sensitive than octane number at octanes in the neighborhood of 100. At intervals tests were made to determine the performance number requirement of the engine, that is, the lowest performance number fuel which could be used to permit acceleration under the foregoing conditions without knocking. Results of these tests are set out in the following table.

Table I

| Hours on test: | Performance number requirement |
|----------------|--------------------------------|
| 0              | 92                             |
| 200            | 107                            |
| 225            | 98.3                           |
| 239            | 98                             |
| 257            | 91.8                           |

As may be seen from the foregoing, 1% propylene carbonate added to the fuel reduced the performance number requirement from 107 to 98.3 within 6 hours, and within 31 hours the requirement had been reduced to the same value as that of a clean engine.

### EXAMPLE II

In this test the Cadillac engine, freshly cleaned, was run for 200 hours on a fuel containing 0.5% of butylene carbonate. A check run of 200 hours was also made using a fuel without butylene carbonate. At the end of the test the engine was taken apart and the deposits were removed, weighed, and examined for their physical properties. It was found that when the fuel contained butylene carbonate the deposits weighed 25 grams, as

compared to 65 grams when the fuel contained no carbonate, and the ignition temperature of the deposits was over 460° C., the upper limit of the testing apparatus, as compared to an ignition temperature of only 164° C. for the deposits formed when the fuel contained no carbonate.

While the foregoing examples were limited to the use of my new fuel compositions in spark ignition engines, the cyclic carbonates are equally effective when added to diesel fuel oils to reduce engine deposits, and the invention should be construed as covering diesel fuel oils containing the carbonates as well as gasolines.

In the appended claims, when the expression "consisting essentially of" is used, it should not be construed as limiting the claimed fuel to a composition containing solely the ingredients named in the claim, but should be construed as covering fuels containing other additives customarily found in commercial fuels, such as gum inhibitors, anti-rust agents, antioxidants and the like, and in addition, in the case of gasoline, anti-knock agents such as tetraethyl lead, and ethylene halide lead scavengers, and in the case of diesel fuel oil, cetane improvers.

This application is a continuation-in-part of my copending application Serial No. 595,055, filed July 2, 1956.

The invention claimed is:

1. A new composition of matter consisting essentially of a normally liquid hydrocarbon internal combustion engine fuel together with a cyclic carbonate inner ester having the formula:



in which R is selected from the group consisting of hydrogen and hydrocarbon radicals, and R' is a hydrocarbon radical, said ester being present in an amount small but sufficient to substantially lessen engine deposit accumulation.

2. The composition of claim 1 in which the ester is propylene carbonate.

3. The composition of claim 1 in which the ester is butylene carbonate.

4. A new composition of matter consisting essentially of a hydrocarbon fraction boiling within the gasoline boiling range, together with a cyclic carbonate inner ester having the formula:



in which R is selected from the group consisting of hydrogen and hydrocarbon radicals, and R' is a hydrocarbon radical, said ester being present in an amount small but sufficient to substantially lessen engine deposit accumulation.

5. The composition of claim 4 in which the ester is propylene carbonate.

6. The composition of claim 4 in which the ester is butylene carbonate.

7. A new composition of matter consisting essentially of a hydrocarbon fraction boiling in the diesel fuel oil range, together with a cyclic carbonate inner ester having the formula:



in which R is selected from the group consisting of hydrogen and hydrocarbon radicals, and R' is a hydrocarbon radical, said ester being present in an amount small but sufficient to substantially lessen engine deposit accumulation.

8. The composition according to claim 7 in which the ester is propylene carbonate.

9. The composition according to claim 7 in which the ester is butylene carbonate.

#### References Cited in the file of this patent

#### UNITED STATES PATENTS

|           |                |               |
|-----------|----------------|---------------|
| 2,334,386 | Gaylor         | Oct. 12, 1943 |
| 2,784,201 | Chitwood       | Mar. 5, 1955  |
| 2,789,891 | Brandes et al. | Apr. 23, 1957 |
| 2,844,450 | Heisler et al. | July 22, 1958 |